



US006177367B1

(12) **United States Patent**  
**Mathis**

(10) **Patent No.:** **US 6,177,367 B1**  
(b4) **Date of Patent:** **Jan. 23, 2001**

(54) **PROCESS FOR PROVIDING FIBERS OR NONWOVENS WITH A HYDROPHILIC COATING**

(75) Inventor: **Raymond Mathis**, Duesseldorf (DE)

(73) Assignee: **Henkel Kommanditgesellschaft auf Aktien**, Duesseldorf (DE)

(\*) Notice: Under 35 U.S.C. 154(b), the term of this patent shall be extended for 0 days.

(21) Appl. No.: **09/230,250**

(22) PCT Filed: **Jul. 15, 1997**

(86) PCT No.: **PCT/EP97/03784**

§ 371 Date: **May 24, 1999**

§ 102(e) Date: **May 24, 1999**

(87) PCT Pub. No.: **WO98/03717**

PCT Pub. Date: **Jan. 29, 1998**

(30) **Foreign Application Priority Data**

Jul. 23, 1996 (DE) ..... 196 29 666

(51) **Int. Cl.<sup>7</sup>** ..... **B32B 27/04**; D06M 13/148; D06M 13/463

(52) **U.S. Cl.** ..... **442/118**; 428/375; 428/396; 427/331; 427/334

(58) **Field of Search** ..... 427/331, 334; 442/118; 428/375, 396

(56) **References Cited**

U.S. PATENT DOCUMENTS

5,045,387 9/1991 Schmalz ..... 428/284

FOREIGN PATENT DOCUMENTS

43 07 186 9/1994 (DE) .

42 43 547 10/1994 (DE) .

0 372 890 6/1990 (EP) .

2 745 013 8/1997 (FR) .

2 185 992 8/1987 (GB) .

OTHER PUBLICATIONS

Ullmann's Encyclopedia of Industrial Chemistry, Fifth Edition (Revised), vol. A17, VCH Weinheim, 1994, pp. 572-583.

Primary Examiner—Elizabeth M. Cole

Assistant Examiner—Ula C. Ruddock

(74) *Attorney, Agent, or Firm*—John E. Drach; Steven J. Trzaska

(57) **ABSTRACT**

A process for making synthetic fibers or nonwoven substrates hydrophilic made from the synthetic fibers comprising applying an effective amount of a finish composition onto the fibers or nonwoven substrates, the finish composition containing: (a) from 50 to 95% by weight of a hydrophobicizing agent selected from the group consisting of at least one quaternary ester amine salt corresponding to formula I:



wherein R<sup>1</sup> is an aliphatic alkyl group containing from 12 to 22 carbon atoms, R<sup>2</sup> is either (CH<sub>2</sub>)<sub>n</sub>—O—COR<sup>1</sup> or an alkyl group containing from 12 to 22 carbon atoms, R<sup>3</sup> and R<sup>4</sup>, independently of one another, represent (CH<sub>2</sub>)<sub>n</sub>—R<sup>5</sup>, where R<sup>5</sup> is H or OH and n is a number from 1 to 3, and X is either a halide, methosulfate, methophosphate or phosphate ion, a quaternary ester amine salt corresponding to formula II:



wherein COR<sup>6</sup> is an aliphatic acyl group containing from 12 to 22 carbon atoms and 0, 1, 2 or 3 double bonds, R<sup>7</sup> is H or OH, n has a value of 1, 2 or 3 and X is either a halide, methosulfate, methophosphate or phosphate ion, and mixtures thereof; and (b) from 5 to 50% by weight of at least one alkyl glycoside corresponding to formula III:



wherein R is a primary linear or methyl-branched aliphatic radical containing from 8 to 22 carbon atoms, G is a glycoside unit containing 5 or 6 carbon atoms and x is a number from 1 to 10, all weights being based on the total weight of the composition.

**20 Claims, No Drawings**

**PROCESS FOR PROVIDING FIBERS OR  
NONWOVENS WITH A HYDROPHILIC  
COATING**

**BACKGROUND OF THE INVENTION**

This invention relates to a process for the hydrophilic finishing of fibers, which exclusively or predominantly contain polyolefins or polyesters, or of nonwovens containing polyolefin or polyester fibers and to fibers or nonwovens which are given a hydrophilic finish by this process.

In the manufacture of sanitary articles, such as diapers or sanitary napkins, absorbent materials are used to absorb aqueous liquids. In order to prevent direct contact with the absorbent material during wear and to increase comfort, the absorbent material is wrapped in a thin water-permeable nonwoven. The nonwovens used for this purpose are normally made of synthetic fibers, such as polyolefin or polyester fibers, because fibers such as these are inexpensive to produce, exhibit good mechanical properties and, in the case of polyolefin, can be heat-bonded. However, untreated polyolefin or polyester fibers are not suitable for this particular application because, in view of their hydrophobic surface, they are not sufficiently permeable to aqueous liquids. Accordingly, the fiber surface has to be made hydrophilic by a corresponding finish. It is also desirable that the hydrophilic finish of the fibers should remain intact for as long as possible without any reduction in the permeability to water of the nonwoven. If nonwovens of the type in question are made up, for example, into diapers, the diapers thus produced can be subjected to repeated stressing without becoming leaky. In this way, the wearing time of the diapers is increased and the waste caused by used diapers can be reduced accordingly.

U.S. Pat. No. 5,045,387 describes, for example, a formulation for the hydrophilic finishing of polyolefin fibers which contains a mixture of an alkoxylated ricinoleic acid derivative, a hydrogenated ricinoleic acid derivative, a C<sub>18</sub> fatty acid and a polyalkoxylated polymethyl siloxane. EP 372 890 B1 discloses fibers which contain polyolefins or polyesters and which have been treated with a finish containing a fatty acid diethanolamide, a polyether-modified silicone, a sorbitan fatty acid ester and a metal salt of an alkyl sulfonate. The disadvantage of finishes such as these lies above all in their high price. In addition, correspondingly finished fibers show poorer behavior in the nonwoven production process, particularly during thermobonding, which results in reduced strength of the nonwoven. According to DE 42 43 547 C2, certain quaternized fatty acid triethanolamine ester salts are suitable for the production of spin finishes for synthetic fibers. These compounds are physiologically safe and show good biodegradability. However, there is nothing in the cited document to suggest that the compounds in question are also suitable for the hydrophilic finishing of synthetic fibers. French patent application 96/2024 discloses water-based preparations with solids contents of 1 to 50% by weight which contain linear saturated fatty alcohols, wax esters, nonionic and/or amphoteric or zwitterionic emulsifiers and cationic surfactants and their use for the production of utility papers with improved softness and as softeners for cellulose and textile fibers.

The problem addressed by the present invention was to provide an improved process for hydrophilically finishing polyolefin- or polyester-containing fibers or nonwovens containing polyolefin or polyester fibers, the hydrophilic finish applied remaining intact, even after repeated wetting.

**BRIEF SUMMARY OF THE INVENTION**

It has now been found that these requirements are satisfied by a process in which the fibers or nonwovens are treated

with a finish which contains quaternary ester amine salts and alkyl glycosides.

Accordingly, the present invention relates to a process for the hydrophilic finishing of fibers, which exclusively or predominantly contain polyolefins or polyesters, or of nonwovens which predominantly contain fibers such as these, characterized in that the nonwovens are treated with an aqueous dispersion of a finish which contains 50 to 95% by weight, based on the total weight of the finish, of at least one 10 quaternary ester amine salt corresponding to formula (I):



in which R<sup>1</sup> is an aliphatic alkyl group containing 12 to 22 carbon atoms, R<sup>2</sup> is either a group (CH<sub>2</sub>)<sub>n</sub>—O—COR<sup>1</sup> or an alkyl group containing 12 to 22 carbon atoms, R<sup>3</sup> and R<sup>4</sup> independently of one another represent a group (CH<sub>2</sub>)<sub>n</sub>—R<sup>5</sup>, where R<sup>5</sup> is H or OH and n is a number of 1 to 3, and X is either a halide, methosulfate, methophosphate or phosphate ion, 5 to 50% by weight of at least one alkyl glycoside corresponding to the general formula RO(G)<sub>x</sub>, in which R is a primary linear or methyl-branched aliphatic radical containing 8 to 22 carbon atoms, G is a glycoside unit containing 5 or 6 carbon atoms and x is a number of 1 to 10, and 30 0 to 30% by weight of glycerol.

**DETAILED DESCRIPTION OF THE  
INVENTION**

The process according to the invention is suitable for fibers which exclusively or predominantly, i.e. more than 50% by weight of which, contain polyolefins or polyesters, and for nonwovens which predominantly contain fibers such as these, fibers exclusively containing polyolefins or polyesters being preferred. Nonwovens containing 100% by weight of polyolefin or polyester fibers are particularly suitable. Polyolefin fibers are among the most commonly used fibers for the production of nonwovens. Examples of suitable polyolefins are polypropylene, polyethylene or copolymers of ethylene or propylene with butadiene. Polyester fibers, mainly polyethylene terephthalate fibers, are also used. Besides the fibers mentioned, other synthetic fibers suitable for the production of nonwovens may also be used, including for example fibers of Nylon®. Fibers consisting of two or more components, for example polyester/copolyester fibers or polypropylene/polyethylene fibers, are also particularly suitable.

The nonwovens used in the process according to the invention may be produced by any of the known processes for producing nonwovens which are described, for example, in Ullmann's Encyclopedia of Industrial Chemistry, Vol. A 17, VCH Weinheim 1994 pages 572-581. Nonwovens produced either by the dry laid process or by the spunbonded process are preferred. The dry laid process starts out from staple fibers which are normally separated by carding into individual fibers and are then laid together by an aerodynamic or hydrodynamic process to form the unbonded nonwoven. The semi-finished nonwoven thus produced is then made up into the final nonwoven by a heat treatment known as thermobonding. To this end, the synthetic fibers are either heated to such an extent that their surface melts and the individual fibers are joined together at their points of contact or the fibers are coated with an additive which melts

during the heat treatment, thus joining the individual fibers to one another. The bonds between the individual fibers are fixed by cooling. Besides this process, any of the other processes known for bonding nonwovens may of course also be used.

By contrast, the spunbonded process starts out from individual filaments which are formed by melt spinning from extruded polymers which are forced under high pressure through spinning jets. The filaments emerging from the spinning jets are bundled, stretched and laid to form a nonwoven which, normally, is then thermobonded.

The process according to the invention is particularly suitable for nonwovens produced by the spunbonded process or by the dry laid process.

In the process according to the invention, the fibers or nonwovens are treated with the finish of quaternary ester amine salt, alkyl glycoside and optionally glycerol by applying the finish to the fibers or to the nonwoven in the form of an aqueous dispersion preferably containing from 5 to 30% by weight of the finish, based on the total weight of the dispersion. Any of the methods and machines typically used in the textiles industry, for example a padding machine, may be used for this purpose. The nonwoven is first contacted with the aqueous dispersion in a bath and the nonwoven thus treated is passed between two rollers, the water being squeezed out by the pressure of the rollers. The process according to the invention is preferably designed in such a way that the fibers or nonwovens receive an add-on of finish in a quantity of 0.3 to 1.5% by weight and, more particularly, in a quantity of 0.5 to 1.0% by weight, based on the weight of the fibers or nonwovens.

The finish used in the process according to the invention contains between 50 and 95% by weight, based on the total weight of the finish, of at least one quaternary ester amine salt corresponding to formula (I). However, finishes containing quaternary ester amine salts corresponding to general formula (II):



in which  $\text{C}\text{OR}^6$  is an aliphatic acyl group containing 12 to 22 carbon atoms and 0, 1, 2 or 3 double bonds,  $\text{R}^7$  is H or OH, n has a value of 1, 2 or 3 and X is either a halide, methosulfate, methophosphate or phosphate ion, are particularly preferred. The compounds corresponding to formula (II) may be obtained, for example, by reaction of diethanol alkyl amines with technical fatty acids and subsequent quaternization. Examples of such compounds are methyl-N-(2-hydroxyethyl)-N,N-di(tallowacyloxyethyl)-ammonium methosulfate and bis-(acyloxyethyl)-hydroxyethyl methylammonium methosulfate. Compounds containing alkyl chains with 16 to 18 carbon atoms and 1 to 3 double bonds are particularly preferred. Mixtures of different ester amine salts corresponding to formulae (I) and/or (II) may also be used.

The finish used in the process according to the invention contains alkyl glycosides corresponding to the general formula  $\text{R}\text{O}(\text{G})_x$ , where R is a primary linear or methyl-branched, more particularly 2-methyl-branched, aliphatic radical containing 8 to 22 and preferably 12 to 18 carbon atoms and G is a glycoside unit containing 5 or 6 carbon atoms, preferably glucose, as an additional component in

quantities of 5 to 50% by weight. The degree of oligomerization x, which represents the distribution of monoglycosides and oligoglycosides, is a number of 1 to 10 and preferably a number of 1.2 to 1.4. Finishes containing alkyl glycosides in quantities of 5 to 30% by weight are particularly preferred.

It has been found that the addition of glycerol in quantities of up to 30% by weight, based on the total weight of the finish used in the process according to the invention, provides the fibers and nonwovens with improved hydrophilic properties and dermatological compatibility. The process according to the invention is preferably carried out by treating the fibers or nonwovens with a glycerol-containing finish which contains glycerol in quantities of 1.0 to 15% by weight, based on the total weight of the finish.

In addition to the compounds described above, other substances known in the textiles field, for example antistatic agents or lubricants, may also be used in the finish. They are normally used in quantities of up to 20% by weight, based on the total weight of the finish.

It can also be of advantage to carry out the process according to the invention by treating the fibers or the nonwovens with a finish which, in addition to the components already described, also contains monoesters of glycerol and a  $\text{C}_{6-14}$  fatty acid in quantities of 5 to 35% by weight, based on the total quantity of the mixture. A particularly preferred monoester is glycerol monolaurate.

In another embodiment, the invention relates to hydrophilic fibers exclusively or predominantly containing polyolefins or polyesters or to nonwovens predominantly containing such fibers which have been produced by the process according to the invention. The fibers or nonwovens show hydrophilic properties which preferably remain intact, even after repeated wetting. In particular, the nonwovens produced in accordance with the invention have liquid strike-through times of less than 10 seconds and, more particularly, less than 5 seconds. In the context of the present invention, liquid strike-through times are understood to be the times which a certain quantity of water or synthetic urine takes to pass through the nonwoven to an absorbent underlayer. This time is determined by EDANA Method No. 150.0-84 (EDANA=European Association of Nonwoven Manufacturers). For use in diapers or similar sanitary articles, the liquid strike-through time should be as short as possible in order to guarantee rapid transport of the liquid through the nonwoven to the absorbent material. In this way, the surface of the nonwoven remains dry and thus leads to increased wearing comfort. The nonwovens produced in accordance with the invention retain this favorable property, even after repeated use, and are further distinguished by the fact that, when the liquid strike-through time is determined by EDANA Method No. 150.0-84 preferably three times and more preferably five times in succession, they always have a liquid strike-through time of less than 10 seconds and, more particularly, less than 5 seconds.

## EXAMPLES

To determine the hydrophilicity of the variously produced nonwovens, the strike-through times of the test nonwovens were measured by EDANA Method No. 150.0-84.

The measurements were carried out using a test instrument with a timer (Lister Tester from Lenzing AG). The test nonwovens (polypropylene spunbonded nonwoven weighing 20 g/m<sup>2</sup>-Lutrasil® 4420 from Freudenberg) were sprayed with an aqueous dispersion of the finish. The test nonwovens were then dried for one hour at 70°C.

For the actual measurements, 6 layers of a filter paper (Evans-Adlard FF3 WIS 150) were placed beneath one layer

of the finished test nonwoven and then contacted with 5 ml of synthetic urine (1000 ml of dist.  $H_2O$ , 9 g NaCl) from the Lister Tester. The measurements were carried out at 20° C./65% relative air humidity. The time which the liquid takes to penetrate through the nonwoven was read off in seconds from the timer.

In order to measure the hydrophilic properties of the nonwovens after repeated stressing, the test nonwoven was placed on a new layer of filter paper after the first measurement without being dried and the measurement was repeated. Times of at most 5 seconds after 5 repetitions were regarded as good. Times of more than 10 seconds were not reproduced.

The results are set out in Table 1 which shows the strike-through times in seconds for nonwovens treated with various finishes (average values of 5 measurements). The nonwovens were coated with 0.5 and 1.0% by weight, based on their weight, of the corresponding finish.

Nonwovens treated with the following finishes were tested. The figures in % by weight are based on the total weight of the finish. The respective finishes were used in the form of an aqueous dispersion containing 20% by weight of active substance, based on the aqueous dispersion.

Finish 1

70% by weight bis-(acyloxyethyl)-hydroxyethyl methylammonium methosulfate

20% by weight  $C_{8-14}$  alkyl polyglucoside

10% by weight glycerol

Finish 2

60% by weight bis-(acyloxyethyl)-hydroxyethyl methylammonium methosulfate

10% by weight  $C_{8-14}$  alkyl polyglucoside

30% by weight glycerol

Finish 3

60% by weight bis-(acyloxyethyl)-hydroxyethyl methylammonium methosulfate

40% by weight  $C_{8-14}$  alkyl polyglucoside

The following finishes were used for comparison:

Finish C1

100% by weight methyl-N-2-hydroxyethyl)-N,N-di(tallowacyloxyethyl)-ammonium methosulfate

Finish C2

50% by weight  $C_{8-14}$  alkyl polyglucoside

50% by weight glycerol

TABLE 1

| Finish              | Number of measurements |      |      |      |      |      |
|---------------------|------------------------|------|------|------|------|------|
|                     | 1                      | 2    | 3    | 4    | 5    | 6    |
| 1<br>(Add-on 0.5%)  | 3.36                   | 3.39 | 3.84 | 4.32 | 5.07 | —    |
| 1<br>(Add-on 1.0%)  | 3.66                   | 4.12 | 3.67 | 3.81 | 4.90 | 5.92 |
| 2<br>(Add-on 0.5%)  | 4.0                    | 3.89 | 4.57 | 5.74 | —    | —    |
| 2<br>(Add-on 1.0%)  | 3.72                   | 3.58 | 3.78 | 4.04 | 5.50 | —    |
| 3<br>(Add-on 0.5%)  | 3.66                   | 3.63 | 4.44 | 6.10 | —    | —    |
| 3<br>(Add-on 1.0%)  | 3.29                   | 3.45 | 4.02 | 4.11 | 5.18 | —    |
| C1<br>(Add-on 0.5%) | 3.26                   | 5.66 | 7.57 | —    | —    | —    |
| C1<br>(Add-on 1.0%) | 3.53                   | 4.66 | 7.41 | 9.93 | —    | —    |

TABLE 1-continued

| Finish              | Number of measurements |      |   |   |   |   |
|---------------------|------------------------|------|---|---|---|---|
|                     | 1                      | 2    | 3 | 4 | 5 | 6 |
| C2<br>(Add-on 0.5%) | 3.34                   | 9.52 | — | — | — | — |
| C2<br>(Add-on 1.0%) | 3.50                   | —    | — | — | — | — |

10 It can be seen that a nonwoven produced in accordance with the invention treated with finish 1 still produces liquid strike-through times of less than 5 seconds at the fourth measurement both with an add-on of 1.0% and with an add-on of 0.5%. This effect is obtained merely with the combination of a quaternized ester amine salt and an alkyl polyglucoside, as the nonwoven treated with finish 3 shows. A nonwoven treated with a commercially available ester ammonium salt, such as finish C1, also shows favorable hydrophilic properties. However, it does not retain these properties as well in the event of repeated stressing, so that the liquid strike-through times become much longer in the following measurements. The nonwoven treated with finish C2 proves that the use of alkyl polyglucoside and glycerol alone does not lead to the required hydrophilic nonwovens. This shows that the required hydrophilic finish is only achieved by the suitable combination of quaternary ester amine salt and alkyl glycosides.

15 What is claimed is:

- 20 30 1. A process for making synthetic fibers or nonwoven substrates hydrophilic made from the synthetic fibers comprising applying an effective amount of a finish composition onto the fibers or nonwoven substrates, the finish composition containing:
- 25 35 (a) from 50 to 95% by weight of a hydrophilic agent selected from the group consisting of at least one quaternary ester amine salt corresponding to formula I:



40 45 50 wherein  $\text{R}^1$  is an aliphatic alkyl group containing from 12 to 22 carbon atoms,  $\text{R}^2$  is either  $(\text{CH}_2)_n - \text{O} - \text{COR}^1$  or an alkyl group containing from 12 to 22 carbon atoms,  $\text{R}^3$  and  $\text{R}^4$ , independently of one another, represent  $(\text{CH}_2)_n - \text{R}^5$ , where  $\text{R}^5$  is H or OH and n is a number from 1 to 3, and X is either a halide, methosulfate, methophosphate or phosphate ion, a quaternary ester amine salt corresponding to formula II:



55 60 65 wherein  $\text{COR}^6$  is an aliphatic acyl group containing from 12 to 22 carbon atoms and 0, 1, 2 or 3 double bonds,  $\text{R}^7$  is H or OH, n has a value of 1, 2 or 3 and X is either a halide, methosulfate, methophosphate or phosphate ion, and mixtures thereof; and

- (b) from 5 to 50% by weight of at least one alkyl glycoside corresponding to formula III:

RO(G)<sub>x</sub>

(III)

wherein R is a primary linear or methyl-branched aliphatic radical containing from 8 to 22 carbon atoms, G is a glycoside unit containing 5 or 6 carbon atoms and x is a number from 1 to 10, all weights being based on the total weight of the composition.

2. The product of the process of claim 1.
3. The process of claim 1 wherein the alkyl glycoside is present in the composition in an amount of from 5 to 30% by weight, based on the weight of the composition.
4. The product of the process of claim 3.
5. The process of claim 1 wherein the finish composition is applied onto the fibers or nonwoven substrates in the form of an aqueous dispersion containing from 5 to 30% by weight of the finish composition, based on the total weight of the aqueous dispersion.
6. The product of the process of claim 5.
7. The process of claim 1 wherein the synthetic fibers are selected from the group consisting of polyolefins, polyesters and mixtures thereof.
8. The product of the process of claim 7.
9. The process of claim 1 wherein the finish composition further contains from 1 to 15% by weight, based on the weight of the composition, of glycerol.
10. The product of the process of claim 9.
11. The process of claim 1 wherein the finish composition further contains up to 20% by weight, based on the weight

of the composition, of an additive selected from the group consisting of an antistatic agent, a lubricant, and mixtures thereof.

12. The product of the process of claim 11.
13. The process of claim 1 wherein the finish composition further contains from 5 to 35% by weight, based on the weight of the composition, of a monoester of glycerol and a C<sub>6-14</sub> fatty acid.
14. The product of the process of claim 13.
15. The process of claim 1 further comprising subsequently applying from 0.3 to 1.5% by weight, based on the weight of the fibers or nonwoven substrates, of the finish composition onto the fibers or nonwoven substrates.
16. The product of the process of claim 15.
17. The process of claim 1 wherein the hydrophilic fibers or nonwoven substrates have a liquid strike-through time of less than 10 seconds, as measured by EDANA Method No. 150.0-8.
18. The product of the process of claim 17.
19. The process of claim 1 wherein the hydrophilic fibers or nonwoven substrates have an average liquid strike-through time of less than 10 seconds, as measured by EDANA Method No. 150.0-8, after three successive measurements.
20. The product of the process of claim 19.

\* \* \* \* \*